# EUROPEAN PATENT SPECIFICATION

(11) **EP 0 490 914 B1**
(45) Date of publication and mention of the grant of the patent: **20.04.1994**
(21) Application number: 90912713.6
(22) Date of filing: 05.09.1990
(51) Int. Cl.: C25D 5/44, C25D 11/18, C23C 18/18

(54) **METHODS FOR DEPOSITING FINISH COATINGS ON SUBSTRATES OF ANODISABLE METALS AND THE PRODUCTS THEREOF**
VERFAHREN ZUR ABLAGERUNG VON DECKSCHICHTEN AUF ANODISIERBAREN METALLSUBSTRATEN UND DADURCH ERHALTENE PRODUKTE
PROCEDES DE DEPOT DE COUCHES DE COUVERTURE SUR DES SUBSTRATS DE METAUX ANODISABLES ET PRODUITS OBTENUS

(30) Priority: 05.09.1989 CA 610259
(43) Date of publication of application: 24.06.1992
(73) Proprietor: ALCAN INTERNATIONAL LIMITED, Montreal, P.Q., H3A 3G1 (CA)
(72) Inventor: FERN, Dan, Kingston, Ontario K7B 6N7 (CA); HANTHORN, Christopher, James, Atlanta, Georgia 30399 (US)
(74) Representative: Pennant, Pyers
(86) International application number: CA9000287
(87) International publication number: WO9103583

(56) References cited:
- EP-A- 0 215 950
- GB-A- 2 123 616
- Chemical Abstracts, vol. 101, No. 26, 24 December 1984, (Columbus, Ohio, US), see page 427, abstract 237330z, & JP-A-59140398 (Pilot Precision Co., Ltd.) 11 August 1984 & Patent Abstracts of Japan, vol. 8, No. 266 (C-255)(1703), 6 December 1984
- S. Wernick et al.: "The Surface Threatment of Aluminium and its Alloys", vol. 1, 5th edition, 1987, Finishing Publications Ltd, (Teddington, Middlesex, GB), pages 329-330

## Description

### Field of the Invention

This invention is concerned with improvements in or relating to methods for depositing metal coatings on substrates of anodisable metals, such as aluminum and its anodisable alloys, and to the products of such methods.

### Review of the Prior Art

The deposition of metals on a substrate, usually steel or aluminum, is a well-developed art. Plating on less easily oxidized metals such as steel is relatively routine, involving for example the deposition of a layer of copper directly on the steel substrate, followed in succession by a thick "semi-bright" nickel layer, a thinner "bright" nickel layer, and an even thinner finish layer of chromium; the chromium is semi-transparent and the bright appearance is actually provided by the bright nickel layer seen through the finish chromium layer.

Plating on anodisable metals, such as aluminum and its anodisable alloys, is considerably more difficult owing to their relative ease of oxidation, and the consequent inevitable presence of an oxide coating which must be removed if adequate adhesion of the deposited layers to the underlying metal substrate is to be obtained. The art currently is dominated by two methods of preparing the substrate surface, namely zincate and stannate immersion. In these processes the substrate surface is immersed in a suitable zincate or stannate solution, usually of the sodium salt, together with other additions that have been found in practice to increase the appearance and adhesion of the coatings. The zinc or tin atoms respectively displace aluminum atoms at the surface, in the process removing the oxide layer, to result in an adherent zinc or tin layer on which other layers, for example copper followed by nickel and chromium can be deposited. Both of these processes are relatively expensive and are therefore mainly used on expensive commodities. The stannate immersion processes are reported to provide better anti-corrosion performance and adhesion of the resultant coatings, but are the more expensive of the two because of the more expensive components and longer processing times.

It has also been proposed to deposit adherent metal coatings directly on aluminum or aluminium alloy substrates by producing a porous anodized layer at the surface of the substrate onto which the subsequent metal layers are deposited; this anodized layer incorporating the oxide layer that was present on the substrate surface. In an article entitled "Plating on Aluminum, a Review" by D.S. Lashmore, published in the June 1985 issue of "Plating & Surface Finishing" (pp 36-39), summarizing previous publications, it was reported that studies have shown that there must be a minimum pore size in the anodized coating, into which the subsequent metal coatings can mechanically "lock" or "key", and that this limits the process to the use of electrolytes that will produce fairly large pores of the order of 0.07 micrometres (700 Angstroms). The report goes on to state it has been found empirically that only anodising solutions comprising phosphoric acid are sucessful, sulfuric or oxalic acid sometimes being mixed with the phosphoric acid. The report further states that the adhesion of the subsequent coatings is primarily mechanical, with the cohesive strength of the porous oxide coatings to the metal substrate being the limiting factor, so that improvements in the anodic process should be directed towards increasing this cohesive strength and the strength of the oxide layer itself. Despite developments of these phosphoric acid anodizing/coating processes for over 50 years they have not yet been widely adopted commercially, apparently because of relatively poor adhesion and brightness.

### Definition of the Invention

It is therefore the principal object of the present invention to provide new methods for plating metal layers on substrates of aluminum and its alloys, and to provide substrates of aluminum and its alloys having metal layers plated thereon by the new methods.

In accordance with the present invention there is provided a new method of depositing metal on a surface of a substrate of an anodisable metal, which substrate has been anodised at the surface using acid to produce a porous anodised layer and subsequently metal has been deposited electrolytically in the pores, the method being characterised by the steps of:
a) anodising the substrate using phosphoric acid to produce a porous anodised layer which is of pore size greater than about 0.03 micrometre and of thickness from about 0.5 to about 50 micrometres;
b) electrolytically depositing pore-filling metal into the pores to adhere to the walls thereof and so as to fill each pore from about 3% to about 30% of its volume; and
c) continuing the deposition of pore-filling metal by electroless deposition on the electrolytically deposited metal to fill each pore to the required extent.

Also in accordance with the invention there is provided a metal plated product consisting of an anodisable metal substrate acid anodised to have a porous anodised layer and having metal electrolytically deposited in the pores thereof characterised in that:
a) the anodised layer is phosphoric acid anodised to have pores of pore size greater than about 0.03 micrometre and to have a thickness of about 0.5 to about 50 micrometres;
b) the porous layer has pore-filling metal electrolytically deposited in the pores thereof so as to adhere to the walls thereof and fill each pore from about 3% to about 30% of its volume; and
c) the porous layer has pore-filling metal electrolessly deposited in the pores on the electrolytically deposited metal so as to fill each pore to the required extent.

### Description of the Drawings

Methods of depositing various layers of metals on a surface of an anodisable substrate, and the products of such methods, constituting particular preferred embodiments of the invention, will now be described by way of example with reference to the accompanying drawings, wherein:-
Figure 1 is a plane cross-section through the surface and adjacent portion of an aluminum substrate, through the porous anodised layer formed thereon by phosphoric acid anodising, and through the various layers of metal that have been deposited on the anodised layer; and
Figure 2 is a plane cross-section to a much enlarged scale of the small portion 2 in Figure 1, showing the anodised layer and the immediately adjacent metal layers.

### Description of the Preferred embodiments

As indicated above, Figure 1 is a cross-section through an aluminum substrate 10 at the upper surface of which there has been formed by acid anodising a layer 12 of aluminum oxide, a portion of which, together with the immediately adjacent portions of the substrate and deposited metal layers, are shown to a larger scale in Figure 2. The anodising employs phosphoric acid which produces elongated wide pores 14 (not seen in Figure 1), and in accordance with this invention at least the bottom portions of the pore walls have had applied thereto by electrolytic deposition a layer of adherent pore-filling metal 16 (also not seen in Figure 1). The electrolytically deposited metal is found initially to deposit principally at the bottoms of the pores and the immediately adjacent parts of the side walls, and the resultant coatings or layers then grow progressively in thickness upwards in the pores as more metal is deposited. It is also found initially that discontinuous patches 17 of the metal are deposited on the side walls in what appears at present to be a random manner. After sufficient metal has been electrolytically deposited the filling of the pores is continued using electroless deposited metal 18 until, in this embodiment, they are completely filled and a continuous support layer has been formed over the entire surface of the anodised layer 12. In this embodiment cobalt is used as the initial electrolytically deposited metal 16 and 17, while electroless nickel is employed for the metal 18. The deposition of metal layers is continued to provide a semi-bright nickel layer 20, a bright nickel layer 22 and a tri-chrome finish layer 24.

The invention thus employs the electrolytic deposition of pore filling metal to apply an inital "seed" coating to the bottom wall portion of each pore and to at least the lower portion of the side wall of each pore. It is found that such an electrolytically deposited metal coating adheres very well to the anodised material, and the subsequently electroless deposited metal adheres very well to the electrolytically deposited metal, whereas metals deposited by electroless processes directly on aluminum oxide do not adhere well and result in lower strength metal coatings. Electroless coating processes have the advantage that they are more efficient than electrolytic processes in filling the pores and result in more dense or compact coatings, and the processes of the invention enable advantage to be taken of this property while overcoming the potential problem of insufficient adherence of the electroless deposited metal to the anodised layer.

The anodised layer is inherently porous in structure because of the manner of its formation, and a typical structure of a layer 12 obtained by phosphoric acid anodising of the aluminum substrate 10 is illustrated by Figure 2. For convenience in drawing the horizontal surfaces of the layers are shown as flat, but in practice they will be seen to be highly irregular even at quite low magnification.

Figure 1 illustrates an embodiment in which an anodised layer 12 of aluminum oxide (Al₂0₃) has been produced of about 2 micrometres (250,000 Angstroms) thickness, typically by use of phosphoric acid at about 20°C and of about 109g/litre or 10% by weight concentration, employing an anodising voltage of about 50-60 volts for 10 minutes. The porous structure obtained is relatively uniform, although highly idealised as shown in Figure 1 for convenience in drawing, and typically the pores 14 will be found to average 0.09 micrometre (900 Angstroms) in transverse dimension, spaced on average about 0.07 micrometre (700 Angstroms) from one another. The pores have an average length/width ratio of 20:1. The bottoms of the pores do not end at the surface of the aluminum substrate, but instead they are on average spaced about 0.07 micrometre (700 Angstroms) from that surface to form a continuous non-porous barrier layer 26 of the relatively non-conductive aluminum oxide, the thickness of this layer depending principally directly on the value of the anodising voltage. It may be noted that references herein and in the literature to pore sizes, etc. are usually made in Angstroms, while references to thicknesses are made in micrometres, merely to avoid the need to refer to large numbers or small fractions, 1 micrometre being equal to 10,000 Angstroms.

It has been found possible in previous commercial practice with sulfuric acid anodising that produces long narrow pores of average transverse dimension 0.015 micrometre (150 Angstroms) to deposit pore filling metal layers that are sufficiently strong and stable of up to about 5 micrometres thickness, but beyond this value the hydrogen that is generated in the long, narrow pores (i.e. length to width ratio of about 330:1) by the electrolytic deposition process tends to cause spalling of the anodised coating, destroying its strength to the extent that it is unsuitable to receive and retain the pore filling metal. Another proolem is that it is difficult to deposit a sufficiently adherent coating of a pore-filling metal into the long narrow pores employing conventional D.C. plating methods. Thus, there is too great a tendency for the plating step to cause physical disruption of the anodised layer, so that the plated metal layer is poorly adherent.

Metal deposition processes may use either alternating current or direct current, or a combination thereof. A.C. deposition is usually much slower that the equivalent D.C. current and D.C. is therefore preferred if speed is important. However, D.C. has a greater tendency to cause disruption of the coating especially with the narrow pores characteristic of sulfuric acid anodising. It is therefore also know to use modified A.C., preferably one in which a predetermind negative-going D.C. has been superimposed on the A.C. Such a system avoids the disruption that would be produced by a pure D.C. current. A.C. produces metal deposition owing to the rectification characteristic of the aluminum oxide, but as the thicknesses of the coatings increase such unmodified A.C. deposition gives poorer pore penetration and slower deposition rates. The D.C. component is therefore increased to the maximum level that does not cause disruption. This method of deposition is disclosed for example in U.S. Patent No. 4,226,680, assigned to Alcan Research and Development Limited, the disclosure of which is incorporated by this reference; these processes have now become known as the Alcan "ANOLOK" (Trade Mark) processes. Other modified A.C. systems are also possible; for example, another system offsets the A.C. waveform in a manner that will produce an effective negative bias, while a further way is to increase the amplitude of the negative portion of the waveform relative to that of the positive portion, which again has the same effect.

The processes of the invention are applicable generally to anodisable metals, their alloys and composites; whether rolled, pressed, cast or wrought. Cast metals are generally less dense and more porous in structure than the corresponding rolled, pressed or wrought product. Attempts to use only electroless deposition, or only electrolytic deposition, directly on the anodised surface of a cast material have not been as successful as the processes of the invention because of this higher porosity and because of the usual higher silicon content (e.g. 7-12%) of such metals. Thus, the more porous metal structure results in anodised layers of lower strength and quality, and electrolytic deposits are more adversely affected by the anodic layer quality than are electroless layers, it is believed because of entrapment of some of the silicon in the barrier layer which interferes with the normal flow of electrons in the deposition current. On the other hand, as explained above, layers applied by direct electroless deposition are generally poorly adherent to the already lower strength anodised layer.

Suitable substrate metals, in addition to aluminum and its anodisable alloys, are magnesium and its anodisable alloys. Metals suitable for the electrolytic deposition of the initial "seed" layer are cobalt, nickel, zinc, copper, tin and palladium. When the substrate is aluminum or an alloy thereof cobalt has been found to be particularly suitable for electrolytic deposition and nickel for electroless deposition.

It is found that as the thickness of the electrolytic layers within the pores increases a point may be reached at which the adhesion to the aluminum begins to decrease, and this then sets an upper limit at which the electrolytic deposition should be stopped and replaced by the electroless deposition. Of course the electrolytic deposition can be discontinued earlier depending upon the other parameters of the particular process. It is found that the thickness of the initial seed coatings, as measured from the bottom of the pores, correlates well with the apparent colour of the substrate surface as seen by an observer, and the table below shows a specific correlation that is obtained when the anodised layer that has been produced by sulfuric acid anodising is 5 micrometres thick; the electrodeposited metal is cobalt. The same principle applies with phosphoric acid anodising but the colours obtained are slightly different. The thickness of the electrolytically deposited metal is most expeditiously expressed in the units milligrams (mg) of metal per square metre (m²) of anodic surface. It is found with this combination that the cut-off for good adhesion is between about 550 and about 850 mg/m².

It will be seen that as little as about 3% will give good adhesion and this is the minimum value for satisfactory results, while at the upper thickness limit of medium bronze for pores of 5 micrometres depth it is estimated that each pore is about 30% filled in volume with the electrolytically deposited metal, leaving the remaining 70% to be filled with the electroless deposited metal. Nickel is found to produce approximately the same colour correlation as cobalt. Copper produces a range of different colours extending from pink through light maroon and dark maroon to black. Tin requires a thicker anodised coating of about 10 micrometres before black is obtained.

The amount of electroless applied metal that is deposited in the pores will of course depend upon the required properties and intended use of the resultant product, and for some applications the pores may not need to be completely filled; from about 6% to about 60% of complete filling may be all that is required. Thus, while a useful range for the electrolytic deposition is about 3% to about 30%, a useful range for the electroless deposition is also from about 3% to the remainder required to fill the pores to the required extent.

Once the initial electrolytic seed deposit and the subsequent electroless deposit have been applied the subsequent processing steps will also depend upon the commercial application of the resultant product and the characteristics and appearance that are required. For example, the electroless deposition can simply be continued until a final layer (over the anodised layer) of adequate thickness is obtained, the usual range for such an application being from about 50 micrometres to about 75 micrometres. More usually the electroless deposition is continued until it forms a support layer of adequate thickness over the entire surface of the anodised layer, as illutrated by Figures 1 and 2, the usual values being from about 0.5 micrometre to about 3 micrometres, more preferably in the range 1-2 micrometres. Thereafter, a finish layer (for example chromium) may be applied over the support layer, with or without the provision of one or more intermediate layers between the support and finish layers.

The use of phosphoric acid is found to be particularly advantageous with cast materials, and it has been found for example that the cast aluminum such as is used for automotive wheels the adhesion of the final coating/s was increased by at least 50% upon use of phosphoric acid in place of sulfuric acid for the anodising. A suitable test for adhesion is to cut the finished part through the substrate and coatings and then to attempt to lift or peel the coating away from the substrate by use of a sharp knife edge; it was found possible with this test to peel the coatings from sulfuric acid anodised substrates with various degrees of difficulty depending on the processing conditions, but not possible to peel it from phosphoric acid anodised substrates.

The use of an anodised layer before plating introduces the possibility, if desired, of a reduction in the thickness of the subsequent plated layers with consequent cost savings. The anodising processes described employing acid baths in the temperature range of 20-35°C are usually characterised as "conventional" anodising, but "hard anodising" processes can also be employed for the invention, the usual bath temperature being in the range 3-7°C; such hard anodised layers are usually thicker than the conventional anodised layers. Further reductions in the subsequent layers therefore are possible by using a thicker and/or stronger anodic film such as that produced using these lower temperature anodising processes. Such hard layers also constitute an excellent basis for the pore-filling metal deposition characteristic of the invention, the electroless layer being the support layer for further deposits, which can be thinner than those normally previously used. It will be understood that this industry is particularly cost conscious, especially with regard to the relatively expensive corrosion-resistant metals that are employed in the intermediate and finish coatings, so that any saving that can be achieved in their thickness for an equivalent performance in protection and/or appearance is commercially important.

In the processes of the invention the anodised layer 10 can be of a thickness in the range 0.5 - 50 micrometres, usually in tne range 1-10 micrometres, preferably in the range 2-6 micrometres, and more preferably 3-5 micrometres, with a thickness of 5 micrometres being usually commercially suitable. The electroless-deposited pore-filling material need not form a support coating of more than about 2 micrometres thickness and excellent results can be obtained with the application of a single thin finish coating of chromium over the support layer. The preferred electroless deposited metal is nickel. Metals otner than nickel, such as cobalt, tin or copper, can also be used. Because of the thin coatings that are employed it is preferred in some processes to pre-treat the surface of the anodisable metal to obtain a very smooth surface; this can be a "macro" treatment by buffing and/or a "micro" treatment of chemical or electro-brightening. The finished chromium layer if provided preferably is of thickness in the range of 0.2-0.3 micrometres.

The invention is further illustrated by the following specific examples:

### Example 1

The process is employed to provide a bright finishing procedure for articles such as cast aluminum automotive wheels, giving a simulation of the appearance of bright chrome or stainless steel, and includes the following steps.
1. An aluminum substrate consisting of cast alloy A413, is pre-treated by cleaning with appropriate alkaline and/or acid solutions, or is pretreated by mechanical buffing.
2. The pretreated substrate is then subjected to a phosphoric acid anodising treatment using acid of 109g/L (10%) concentration by weight at 21°C; the anodising is begun at 60VDC for 30 minutes and is then ramped down to approximately 18 VDC for about 0.5 minute.
3. The anodised substrate has the initial "seed" electrolytic coating of cobalt applied using a cobalt-based "ANOLOK" (trade mark) electrolyte as disclosed in U.S. Patent No. 3,616,309 at 21°C and 12.5 V.A.C., with or without up to 4 V.D.C. bias. The electolytic deposition proceeds for a period of about one minute.
4. A pore-filling coating of nickel is then applied by immersion in an electroless nickel solution (Harshaw "Alpha 103B" - trade mark) for 20 minutes at pH4.7 and temperature 93°C, thus completely filling the pores and forming a support coating of about 0.5 to about 3.0 micrometres thickness
5. The support layer is coated with an electrolytically-deposited semi-bright layer of nickel of about 10 micrometres thickness using Harshaw "PERFLOW" (trade mark) semi-bright solution at pH4.3; temperature 57°C; current density 5 amps per square decimetre (A/dm²); and for a period of thirty/minutes.
6. The semi-bright layer is coated with a bright layer of nickel of about 10 micrometres thickness using Harshaw "SUPREME" (trade mark) bright solution at pH4.0; temperature 66°C; current density 4A/dm² and period 10 minutes.
7. The example is completed by electrolytically depositing a trichrome finish layer using Harshaw "TRI-CHROME PLUS" (trade mark) solution at pH2.7; temperature 30°C; current density 10 A/dm² for 5 minutes.

During the process the substrate will be rinsed in known manner which need not be detailed here. It may be noted that in this and the other examples described a cyanide or hexavalent chromium bath is not used, which is environmentally desirable.

## Claims

1. A method of depositing metal on a surface of a substrate of an anodisable metal, which substrate has been anodised at the surface using acid to produce a porous anodised layer and subsequently metal has been deposited electrolytically in the pores, the method being characterized by the steps of:
a) anodising the substrate using phosphoric acid to produce a porous anodised layer which is of pore size greater than about 0.03 micrometre and of thickness from about 0.5 to about 50 micrometres;
b) electrolytically depositing pore-filling metal into the pores to adhere to the walls thereof and so as to fill each pore from about 3% to about 30% of its volume; and
c) continuing the deposition of pore-filling metal by electroless deposition on the electrolytically deposited metal to fill each pore to the required extent.

2. A method as claimed in claim 1, characterised in that the anodisation produces pores of transverse dimension from about 0.03 to 0.10 micrometre.

3. A method as claimed in claim 1 or 2, characterised in that the electrolytic deposition is continued to a cut-off value at which adhesion of the metal begins to decrease.

4. A method as claimed in claim 3, characterised in that the electrolytically deposited pore-filling metal is deposited to a thickness of up to 550 milligrams per square metre.

5. A method as claimed in any one of claims 1 to 4, characterised in that the electroless deposition is continued until a coating of the metal of thickness in the range about 0.5 to 3 micrometres is deposited on the surface of the anodised layer.

6. A method as claimed in claim 5, characterised in that the electroless deposited metal is deposited to form a support layer on the surface of the substrate of a thickness in the range of about 0.5 to 3 micrometres, and in that one of more subsequent layers are deposited on the support layer.

7. A method as claimed in any one of claims 1 to 4, characterized in that the electroless deposited metal is deposited to a thickness of about 10-25 micrometres on the surface of the substrate.

8. A method as claimed in any one of claims 1 to 7, characterised in that the anodisable substrate metal is selected from aluminum and magnesium and anodisable alloys thereof.

9. A method as claimed in any one of claims 1 to 7, characterised in that the anodisable metal is selected from cast aluminum and its alloys.

10. A method as claimed in any one of claims 1 to 9, characterised in that the electrolytically deposited pore-filling metal is selected from nickel, cobalt, zinc, copper, tin, palladium and mixtures thereof.

11. A method as claimed in any one of claims 1 to 10, characterised in that the electroless pore-filling metal is selected from nickel, cobalt, copper, tin and mixtures thereof.

12. A metal plated product consisting of an anodisable metal substrate acid anodised to have a porous anodised layer and having metal electrolytically deposited in the pores therof characterised in that:
a) the anodised layer is phosphoric acid anodised to have pores of pore size greater than about 0.03 micrometre and to have a thickness of about 0.5 to about 50 micrometres;
b) the porous layer has a pore-filling metal electrolytically deposited in the pores thereof so as to adhere to the walls, thereof and fill each pore from about 3% to about 30% of its volume; and
c) the porous layer has pore-filling metal electrolessly deposited in the pores on the electrolytically deposited metal so as to fill each pore to the required extent.

13. A product as claimed in claim 12, characterised in that the substrate has been anodised to produce pores of transverse dimension from about 0.03 to 0.10 micrometre.

14. A product as claimed in claim 12 or 13, characterised in that tne electrolytically deposited pore-filling metal is deposited to a thickness of up to 550 milligrams per square metre.

15. A product as claimed in any one of claims 12 to 13 characterised in that the electroless metal is sufficiently thick to form a coating deposited on the surface of the anodised layer.

16. A product as claimed in claim 15, characterised in that the electroless deposited metal is deposited to a thickness of about 10-25 micrometres on the surface of the substrate.

17. A product as claimed in any one of claims 12 to 15, characterised in that the electroless deposited metal is deposited to form a support layer on the surface of the substrate of a thickness in the range of about 0.5 to 3 micrometres, and in that one or more subsequent layers are deposited on the support layer.

18. A product as claimed in any one of claims 12 to 17, characterised in that the anodisable substrate metal is selected from aluminum and magnesium and anodisable alloys thereof.

19. A product as claimed in any one of claims 12 to 17, characterised in that the anodisable metal is selected from cast aluminium and its alloys.

20. A product as claimed in any one of claims 12 to 19, characterised in that the electrolytically deposited pore-filling metal is selected from nickel, cobalt, zinc, copper, tin, palladium and mixtures thereof.

21. A product as claimed in any one of claims 12 to 20, characterised in that the electroless pore-filling metal is selected from nickel, cobalt, copper, tin and mixtures thereof.

## Patentansprüche

1. Ein Verfahren zur Abscheidung von Metall auf einer Oberfläche eines Substrats aus einem anodisierbaren Metall, wobei dieses Substrat unter Verwendung von Säure an der Oberfläche anodisiert worden ist, um eine poröse anodisierte Schicht zu erzeugen, und anschließend Metall elektrolytisch in den Poren abgeschieden worden ist, wobei das Verfahren durch die Schritte gekennzeichnet ist:
a) Anodisieren des Substrats unter Verwendung von Phosphorsäure, um eine poröse anodisierte Schicht zu erzeugen, die eine Porengröße von mehr als etwa 0,03 Mikrometern und eine Dicke von etwa 0,5 bis etwa 50 Mikrometern aufweist;
b) elektrolytisches Abscheiden von Porenfüllmetall in die Poren, so daß dieses an den Wänden derselben anhaftet und jede Pore zu etwa 3% bis etwa 30% ihres Volumens füllt; und
c) Fortsetzen der Abscheidung von Porenfüllmetall durch stromlose Abscheidung auf dem elektrolytisch abgeschiedenen Metall, um jede Pore bis zum erforderlichen Umfang zu füllen.

2. Ein Verfahren nach Anspruch 1, dadurch gekennzeichnet, daß die Anodisierung Poren mit einer Querabmessung von etwa 0,03 bis 0,10 Mikrometern erzeugt.

3. Ein Verfahren nach Anspruch 1 oder 2, dadurch gekennzeichnet, daß die elektrolytische Abscheidung bis zu einem Abschlußwert fortgesetzt wird, bei dem die Adhäsion des Metalls beginnt abzunehmen.

4. Ein Verfahren nach Anspruch 3, dadurch gekennzeichnet, daß das elektrolytisch abgeschiedene Porenfüllmetall bis zu einer Dicke von bis zu 550 Milligramm pro Quadratmeter abgeschieden wird.

5. Ein Verfahren nach einem der Ansprüche 1 bis 4, dadurch gekennzeichnet, daß die stromlose Abscheidung fortgesetzt wird, bis ein Überzug des Metalls mit einer Dicke im Bereich von etwa 0,5 bis 3 Mikrometern auf der Oberfläche der anodisierten Schicht abgeschieden ist.

6. Ein Verfahren nach Anspruch 5, dadurch gekennzeichnet, daß das elektrolytisch abgeschiedene Metall abgeschieden wird, um eine Trägerschicht auf der Oberfläche des Substrats mit einer Dicke im Bereich von etwa 0,5 bis 3 Mikrometern zu bilden, und daß eines oder mehrere folgende Schichten auf der Trägerschicht abgeschieden werden.

7. Ein Verfahren nach einem der Ansprüche 1 bis 4, dadurch gekennzeichnet, daß das stromlose abgeschiedene Metall bis zu einer Dicke von etwa 10-25 Mikrometern auf der Oberfläche des Substrats abgeschieden wird.

8. Ein Verfahren nach einem der Ansprüche 1 bis 7, dadurch gekennzeichnet, daß das anodisierbare Substratmetall ausgewählt wird aus Aluminium und Magnesium und anodisierbaren Legierungen derselben.

9. Ein Verfahren nach einem der Ansprüche 1 bis 7, dadurch gekennzeichnet, daß das anodisierbare Metall ausgewählt wird aus Gußaluminium und seinen Legierungen.

10. Ein Verfahren nach einem der Ansprüche 1 bis 9, dadurch gekennzeichnet, daß das elektrolytisch abgeschiedene Porenfüllmetall ausgewählt wird aus Nickel, Kobalt, Zink, Kupfer, Zinn, Palladium und Mischungen derselben.

11. Ein Verfahren nach einem der Ansprüche 1 bis 10, dadurch gekennzeichnet, daß das stromlose Porenfüllmetall ausgewählt wird aus Nickel, Kobalt, Kupfer, Zinn und Mischungen derselben.

12. Ein mit Metallüberzug versehenes Produkt, das aus einem anodisierbaren Metallsubstrat besteht, das mit Säure anodisiert ist, um eine poröse anodisierte Schicht aufzuweisen, und mit elektrolytisch in den Poren derselben abgeschiedenem Metall, dadurch gekennzeichnet, daß:
a) die anodisierte Schicht mit Phosphorsäure anodisiert ist, um Poren einer Porengröße von mehr als 0,03 Mikrometern und eine Dicke von etwa 0,5 bis etwa 50 Mikrometern aufzuweisen;
b) die poröse Schicht ein in den Poren derselben elektrolytisch abgeschiedenes Porenfüllmetall aufweist, welches an den Wänden derselben anhaftet und jede Pore zu etwa 3% bis etwa 30% ihres Volumens füllt; und
c) die poröse Schicht in den Poren auf dem elektrolytisch abgeschiedenen Metall stromlos abgeschiedenes Porenfüllmetall aufweist, um jede Pore bis zum erforderlichen Umfang zu füllen.

13. Ein Produkt nach Anspruch 12, dadurch gekennzeichnet, daß das Substrat anodisiert worden ist, um Poren mit einer Querabmessung von etwa 0,03 bis 0,10 Mikrometern zu erzeugen.

14. Ein Produkt nach Anspruch 12 oder 13, dadurch gekennzeichnet, daß das elektrolytisch abgeschiedene Porenfüllmetall bis zu einer Dicke von bis zu 550 Milligramm pro Quadratmeter abgeschieden ist.

15. Ein Produkt nach einem der Ansprüche 12 bis 13, dadurch gekennzeichnet, daß das stromlose Metall genügend dick ist, um einen auf der Oberfläche der anodisierten Schicht abgeschiedenen Überzug zu bilden.

16. Ein Produkt nach Anspruch 15, dadurch gekennzeichnet, daß das stromlos abgeschiedene Metall bis zu einer Dicke von etwa 10-25 Mikrometern auf der Oberfläche des Substrats abgeschieden ist.

17. Ein Produkt nach einem der Ansprüche 12 bis 15, dadurch gekennzeichnet, daß das stromlos abgeschiedene Metall abgeschieden ist, um eine Trägerschicht auf der Oberfläche des Substrats mit einer Dicke im Bereich von etwa 0,5 bis 3 Mikrometern zu bilden, und daß eine oder mehrere folgende Schichten auf der Trägerschicht abgeschieden sind.

18. Ein Produkt nach einem der Ansprüche 12 bis 17, dadurch gekennzeichnet, daß das anodisierbare Substratmetall ausgewählt ist aus Aluminium und Magnesium und anodisierbaren Legierungen derselben.

19. Ein Produkt nach einem der Ansprüche 12 bis 17, dadurch gekennzeichnet, daß das anodisierbare Metall ausgewählt ist aus Gußaluminium und seinen Legierungen.

20. Ein Produkt nach einem der Ansprüche 12 bis 19, dadurch gekennzeichnet, daß das elektrolytisch abgeschiedene Porenfüllmetall ausgewählt ist aus Nickel, Kobalt, Zink, Kupfer, Zinn, Palladium und Mischungen derselben.

21. Ein Produkt nach einem der Ansprüche 12 bis 20, dadurch gekennzeichnet, daß das stromlose Porenfüllmetall ausgewählt ist aus Nickel, Kobalt, Kupfer, Zinn und Mischungen derselben.

## Revendications

1. Procédé pour déposer un métal sur la surface d'un substrat en un métal anodisable, lequel substrat a été anodisé sur sa surface en utilisant un acide pour produire une couche anodisée poreuse et dans lequel on a déposé ultérieurement un métal électrolytiquement dans les pores, le procédé étant caractérisé par les étapes suivantes :
a) anodiser le substrat en utilisant de l'acide phosphorique pour obtenir une couche anodisée poreuse, dont la dimension de pores est supérieure à environ 0,03 micromètre et qui a une épaisseur d'environ 0,5 à environ 50 micromètres;
b) déposer électrolytiquement dans les pores un métal de remplissage des pores pour adhérer aux parois de ces pores et remplir ainsi chaque pore d'environ 3% à environ 30% de son volume; et
c) continuer le dépôt de métal de remplissage des pores par dépôt sans courant sur le métal déposé électrolytiquement pour remplir chaque pore au volume requis.

2. Procédé selon la revendication 1, caractérisé en ce que l'anodisation produit des pores dont la dimension transversale est comprise entre environ 0,03 et 0,10 micromètre.

3. Procédé selon la revendication 1 ou 2, caractérisé en ce que le dépôt électrolytique continue jusqu'à une valeur d'interruption pour laquelle l'adhérence du métal commence à diminuer.

4. Procédé selon la revendication 3, caractérisé en ce que le métal de remplissage des pores déposé électrolytiquement est déposé jusqu'à une épaisseur de 550 mg/m2.

5. Procédé selon l'une des revendications 1 à 4, caractérisé en ce que le dépôt sans courant continue jusqu'à ce qu'un revêtement de métal ayant une épaisseur comprise entre environ 0,5 et 3 micromètres soit déposé sur la surface de la couche anodisée.

6. Procédé selon la revendication 5, caractérisé en ce que le métal déposé sans courant est déposé pour former une couche support sur la surface du substrat d'une épaisseur comprise entre environ 0,5 et 3 micromètres et en ce qu'une ou plusieurs couches ultérieures sont déposées sur la couche support.

7. Procédé selon l'une des revendications 1 à 4, caractérisé en ce que le métal déposé sans courant est déposé jusqu'à une épaisseur d'environ 10 à 25 micromètres sur la surface du substrat.

8. Procédé selon l'une des revendications 1 à 7, caractérisé en ce que le métal du substrat anodisable est choisi parmi l'aluminium et le magnésium et leurs alliages anodisables.

9. Procédé selon l'une des revendications 1 à 7, caractérisé en ce que le métal anodisable est choisi parmi l'aluminium coulé et ses alliages.

10. Procédé selon l'une des revendications 1 à 9, caractérisé en ce que le métal de remplissage des pores déposé électrolytiquement est choisi parmi le nickel, le cobalt, le zinc, le cuivre, l'étain, le palladium et leurs mélanges.

11. Procédé selon l'une des revendications 1 à 10, caractérisé en ce que le métal de remplissage des pores sans courant est choisi parmi le nickel, le cobalt, le cuivre, l'étain et leurs mélanges.

12. Produit plaqué métal constitué par un substrat métallique anodisable anodisé à l'acide pour avoir une couche anodisée poreuse et ayant un métal déposé électrolytiquement dans les pores de cette couche, caractérisé en ce que :
a) la couche anodisée est anodisée à l'acide phosphorique pour avoir des pores dont la dimension est supérieure à environ 0,03 micromètre et qui a une épaisseur d'environ 0,5 à environ 50 micromètres;
b) la couche poreuse a un métal de remplissage des pores déposé électrolytiquement dans les pores pour adhérer aux parois de ceux-ci et remplir chaque pore d'environ 3% à environ 30% de son volume; et
c) la couche poreuse a un métal de remplissage des pores déposé sans courant dans les pores sur le métal déposé électrolytiquement de façon à remplir chaque pore au volume requis.

13. Produit selon la revendication 12, caractérisé en ce que le substrat a été anodisé pour produire des pores ayant une dimension transversale d'environ 0,03 à 0,10 micromètre.

14. Produit selon la revendication 12 ou 13, caractérisé en ce que le métal de remplissage des pores déposé électrolytiquement est déposé à une épaisseur pouvant atteindre 550 mg/m2.

15. Produit selon l'une des revendications 12 et 13, caractérisé en ce que le métal déposé sans courant est suffisamment épais pour former un revêtement déposé sur la surface de la couche anodisée.

16. Produit selon la revendication 15, caractérisé en ce que le métal déposé sans courant est déposé jusqu'à une épaisseur d'environ 10 à 25 micromètres sur la surface du substrat.

17. Produit selon l'une des revendications 12 à 15, caractérisé en ce que le métal déposé sans courant est déposé pour former une couche support sur la surface du substrat ayant une épaisseur comprise entre environ 0,5 et 3 micromètres et en ce qu'une ou plusieurs couches ultérieures sont déposées sur la couche support.

18. Produit selon l'une des revendications 12 à 17, caractérisé en ce que le métal du substrat anodisable est choisi parmi l'aluminium et le magnésium et leurs alliages anodisables.

19. Produit selon l'une des revendications 12 à 17, caractérisé en ce que le métal anodisable est choisi parmi l'aluminium coulé et ses alliages.

20. Produit selon l'une des revendications 12 à 19, caractérisé en ce que le métal de remplissage des pores déposé électrolytiquement est choisi parmi le nickel, le cobalt, le zinc, le cuivre, l'étain, le palladium et leurs mélanges.

21. Produit selon l'une des revendications 12 à 20, caractérisé en ce que le métal de remplissage des pores déposé sans courant est choisi parmi le nickel, le cobalt, le cuivre, l'étain et leurs mélanges.
